

99

Patented Dec. 13, 1932

1,890,453

## UNITED STATES PATENT OFFICE

FREDERIC CHARLES BOWMAN, OF LOS ANGELES, CALIFORNIA, ASSIGNOR TO A. E. MAAS CHEMICAL CO., OF LOS ANGELES, CALIFORNIA, A CORPORATION OF CALIFORNIA

## TRISODIUM PHOSPHATE-SODIUM NITRATE

No Drawing.

Application filed August 24, 1931. Serial No. 559,138.

This invention relates to a trisodium phosphate-sodium nitrate and to the method of preparing compounds of trisodium phosphate and sodium nitrate wherein the sodium nitrate is substituted in the sodium phosphate for sodium hydroxide.

Trisodium phosphate in its commercial form contains free sodium hydroxide and as sold commercially has the exceedingly great 10 disadvantage of caking readily at ordinary summer temperatures. The free sodium hydroxide carried by the commercial trisodium phosphate also produces a further disadvantage in the production of solutions which are 15 of strongly irritating character due to the presence of the free sodium hydroxide so that strong solutions of the trisodium phosphate containing free sodium hydroxide can not be utilized without considerable irritation to the 20 skin of the hands or other portions of the body contacted by the solution.

In the preparation of a non-caking, non-irritating form of sodium phosphate, I have found that trisodium phosphate, which is generally assigned the chemical formula of



as it appears in the commercial salt, contains 2 to 3% excess sodium hydroxide, and that 20 this sodium hydroxide is actually present in the crystalline form of the trisodium phosphate as substituted in part for one molecule of the twelve molecules of water of crystallization given in the above formula.

35 I have determined that ordinary trisodium phosphate is a variable solid solution of probably two forms of trisodium phosphate, the variable solid solution of these two forms being apparently a mixture of



indicating that all or part of one of the twelve waters of crystallization may be replaced or is replaced by  $\frac{1}{4}$  mol. of sodium hydroxide.

45 I have found that this sodium hydroxide which has apparently replaced a portion of one of the waters of crystallization of the commercial trisodium phosphate may be itself substituted in the crystal form by sodium nitrate so that the resultant compound of tri-

sodium phosphate-sodium nitrate does not have the caking properties of the ordinary trisodium phosphate-sodium hydroxide, and does not have the skin irritating properties of the trisodium phosphate containing free sodium hydroxide.

The chemical formula of the trisodium phosphate-sodium nitrate may perhaps be best expressed in the crystal form which it takes when the substitution of sodium nitrate for sodium hydroxide has been carried to its practical limit as



I have found that no excess of nitrate, however great, will push the sodium nitrate content of the crystals above 5.6%. The formula



has a theoretical sodium nitrate content of 5.55%  $\text{NaNO}_3$  indicating that when a large excess of sodium nitrate is utilized, the substitution of sodium nitrate for sodium hydroxide may be carried to completion, and that the sodium nitrate will completely be substituted for the sodium hydroxide present in the ordinary commercial form of trisodium phosphate.

I have found that to carry the sodium nitrate content of the trisodium phosphate-sodium nitrate compound to over 4% sodium nitrate requires the use of too great an excess of sodium nitrate in the crystallizing solution in order to be commercially feasible, and that when approximately 3% sodium nitrate is substituted into commercial trisodium phosphate for the sodium hydroxide thereof, the resultant compounds, which may be defined as trisodium phosphate-sodium nitrate-sodium hydroxide, plus the water of crystallization, gives to the resultant compound the qualities desired of reducing the irritating property of the ordinary trisodium phosphate, and eliminates to a satisfactory degree the caking property of the trisodium phosphate containing all free sodium hydroxide.

In the preparation of the complex salt of trisodium phosphate and sodium nitrate, I have found that the sodium nitrate is substituted for the sodium hydroxide to a practical

extent only when there is employed a comparatively high excess of sodium nitrate in the crystallizing solution formed by the dissolving of sodium nitrate and trisodium phosphate.

I have also found that if the alkalinity of this crystallizing solution is too high, or there is too great an excess of free sodium hydroxide or alkali in the crystallizing solution, that 10 the substitution of sodium nitrate for the sodium hydroxide will not take place to any marked or practical extent.

In considering the alkalinity of the crystallizing solution, it is most convenient to express this alkalinity as "alkaline ratio", which 15 is the ratio of titration with phenolphthalein to the further titration with methyl orange. Trisodium phosphate has therefore a ratio or alkaline ratio of 1.

20 The best ratio or alkaline ratio for the crystallizing liquor I have found is approximately 1. The effect of increased alkaline ratio for a given excess of sodium nitrate in a crystallizing liquor is shown by the following table:

Table A

| Experiment No.                  | 1      | 2      | 3      |
|---------------------------------|--------|--------|--------|
| Ratio of crystallizing liquor   | 0.50   | 1.00   | 1.49   |
| Ratio of mother liquor          | 0.39   | 0.526  | 4.36   |
| Analysis of crystals:           |        |        |        |
| Ratio                           | 1.035  | 1.072  | 1.283  |
| Na <sub>3</sub> PO <sub>4</sub> | 43.23% | 41.26% | 41.35% |
| NaNO <sub>3</sub>               | 4.00%  | 4.16%  | 0.10%  |
| NaOH                            | 0.22%  | 0.7%   | 2.85%  |

30 The low nitrate content of the crystals in Experiment No. 3 was partly due to the fact that only one-half as great an excess of sodium nitrate was present as in the other two experiments. In Experiment No. 1, at the end of crystallization crystals of disodium phosphate began to be formed.

40 The effect of the concentration or excess 45 of sodium nitrate in the crystallizing liquor is shown by the following table:

Table B

| Experiment No.                                               | 1     | 2     | 3     | 4     | 5     |
|--------------------------------------------------------------|-------|-------|-------|-------|-------|
| NaNO <sub>3</sub> :P <sub>2</sub> O <sub>5</sub> in liquor   | 0.05  | 0.08  | 0.79  | 1.88  | 2.84  |
| NaNO <sub>3</sub> :P <sub>2</sub> O <sub>5</sub> in crystals | 0.02  | 0.04  | 0.21  | 0.22  | 0.31  |
| NaNO <sub>3</sub> in crystals                                | 0.40% | 0.65% | 4.00% | 4.04% | 5.84% |

50 The sodium nitrate content of the crystals in Experiment No. 5, which is slightly higher than the theoretical maximum of 5.55%, is accounted for by contamination of the crystals with mother liquor.

55 The effect of recrystallization of trisodium phosphate-sodium nitrate shows clearly that the alkaline ratio of the crystals is progressively increased. This effect is shown in the 60 following table, wherein there is illustrated

the successive recrystallization five times of a lot of trisodium phosphate-sodium nitrate:

Table C

| Crop No.          | 1     | 2     | 3     | 4     | 5     | 70 |
|-------------------|-------|-------|-------|-------|-------|----|
| NaNO <sub>3</sub> | 3.14% | 2.60% | 1.26% | 0.42% | 0.05% |    |
| Alkaline ratio    | 1.030 | 1.056 | 1.132 | 1.159 | 1.193 |    |

This table shows that successive recrystallizations from water gradually remove the nitrate content of the compound and replace it with the hydroxide so that finally trisodium phosphate of standard alkalinity is attained.

60 From the foregoing tables it will be evident that the composition of the trisodium phosphate-sodium nitrate varies within the following limits:

| Per cent                                                           |
|--------------------------------------------------------------------|
| Sodium phosphate (Na <sub>3</sub> PO <sub>4</sub> ) - 41.1 to 43.6 |
| Sodium nitrate (NaNO <sub>3</sub> ) - 5.55 to 0.08                 |
| Sodium hydroxide (NaOH) - 0.22 to 2.85                             |

65 the balance being in each case the water of crystallization.

An analysis of Experiment No. 5, shown in Table B, showed

| Per cent                                    |
|---------------------------------------------|
| Sodium phosphate - 42.55                    |
| Sodium nitrate - 5.84                       |
| Loss on ignition - 50.12                    |
| Sodium hydroxide and unaccounted for - 1.49 |

70 Expressed in molecules, this is:

|                              |      |
|------------------------------|------|
| Trisodium phosphate          | 4.00 |
| Sodium nitrate               | 1.06 |
| H <sub>2</sub> O by ignition | 44.4 |

75 The chemical formula of trisodium phosphate-sodium nitrate or trisodium phosphate-sodium nitrate-sodium hydroxide in crystalline form as shown by this experiment is:



80 In the preparation of the trisodium phosphate-sodium nitrate compounds, I have also discovered that not only may complex salt of sodium phosphate-sodium nitrate and sodium hydroxide be formed, but other complex salt may be formed wherein sodium nitrate is partially substituted for the sodium hydroxide contained in the commercial form of trisodium phosphate, for example, mixtures of sodium salts of monobasic acids such as sodium chloride or the like may be substituted with sodium nitrate for a portion of the sodium hydroxide which has apparently displaced one of the waters of crystallization of the commercial form of trisodium phosphate.

85 I have found, for example, that trisodium phosphate-sodium nitrate-sodium chloride-sodium hydroxide may be formed 120

having in percent substantially the following composition:

|                                 | Per cent |
|---------------------------------|----------|
| Na <sub>3</sub> PO <sub>4</sub> | 40.82    |
| NaOH                            | 1.21     |
| 5 NaCl                          | 2.00     |
| NaNO <sub>3</sub>               | 0.92     |
| H <sub>2</sub> O by difference  | 54.95    |

showing that the salts of the dodecahydrate series form solid solutions with each other freely, and a salts of even greater complexity could be built up if desired.

In carrying out the method embodying my invention for the formation of sodium phosphate-sodium nitrate compounds, I prefer to proceed as follows:

For example, commercial trisodium phosphate is dissolved with sodium nitrate in water, and the composition of the crystallizing liquor is determined. In dissolving the trisodium phosphate and the sodium nitrate in water, heat is applied so that the salts dissolve.

In order to maintain the correct alkalinity ratio of approximately 1, the following illustrative example of an actual production of trisodium phosphate-sodium nitrate is given:

|                                                     | Grams |
|-----------------------------------------------------|-------|
| Commercial trisodium phosphate                      | 1200  |
| 30 Commercial 26° Baumé disodium phosphate solution | 488   |
| Commercial sodium nitrate                           | 154   |

were dissolved by heating in a large evaporating dish in 1000 grams of water. The composition of the batch was then determined to be

|                               | Grams per c. c. |
|-------------------------------|-----------------|
| P <sub>2</sub> O <sub>5</sub> | 0.138           |
| NaNO <sub>3</sub>             | 0.07            |

and the alkalinity ratio of the solution of crystallizing liquor was 1.00.

The batch was cooled with occasional stirring and allowed to stand. Needle crystals began to form when the batch had cooled to 71° C., and when the temperature of the batch had fallen to 60° C., there was a large crop of crystals. After continued cooling, a heavy crop of crystals was filtered from the solution, washed with dilute alcohol, then with strong alcohol, and finally dried in a thin layer for several hours at approximately 20° C. The crystals produced were fine, glistening hexagonal crystals which, on analysis showed

|                                   | Per cent |
|-----------------------------------|----------|
| Na <sub>3</sub> PO <sub>4</sub>   | 41.1     |
| NaNO <sub>3</sub>                 | 4.06     |
| Free NaOH                         | 0.9      |
| 60 H <sub>2</sub> O by difference | 53.94    |

In carrying out the process commercially it has been found that the alkalinity of the crystallizing liquor controls the size of the crystals that are formed and that there is

little latitude in the alkalinity required for the production of marketable crystals. A representative factory run given, for example, is:

| Crystallizing liquor            | 70         |
|---------------------------------|------------|
| Volume                          | 3000 gals. |
| Baumé                           | 30.5°      |
| Temp.                           | 114° C.    |
| Na <sub>3</sub> PO <sub>4</sub> | 12.65%     |
| NaNO <sub>3</sub>               | 9.26%      |
| NaOH                            | 0.32%      |
| Alkaline ratio                  | 1.10       |

| Crystals produced               | 80        |
|---------------------------------|-----------|
| Weight                          | 9100 lbs. |
| Na <sub>3</sub> PO <sub>4</sub> | 43.59%    |
| NaNO <sub>3</sub>               | 3.32%     |
| NaOH                            | 0.56%     |
| Alkaline ratio                  | 1.05      |

The mother liquor was analyzed and showed the following:

2100 gallons having a specific gravity of 23.50° Baumé at a temperature of 27° C., and containing

|                                 |       |
|---------------------------------|-------|
| Na <sub>3</sub> PO <sub>4</sub> | 6.24% |
| NaNO <sub>3</sub>               | 10.9% |
| Alkaline ratio                  | 1.07  |

In crystallizing the crystals from the mother liquor, the crystallizing liquor was placed in a stirred water-cooled crystallizer over night. The crystals were then centrifuged, washed and dried at about 38° C., and barrelled.

Having fully described my invention, it is to be understood that I do not wish to be limited to the details herein set forth, but my invention is of the full scope of the appended claims.

I claim:

1. The herein described composition of matter consisting of a compound of sodium phosphate and sodium nitrate.
2. The herein described composition of matter consisting of a compound of trisodium phosphate and sodium nitrate.
3. The herein described composition of matter consisting of a compound of trisodium phosphate and sodium nitrate in crystalline form.
4. The herein described trisodium phosphate composition containing not less than .08% sodium nitrate.
5. The herein described trisodium phosphate composition containing approximately .08% to 5.55% sodium nitrate.
6. The herein described composition of matter having a formula



7. The herein described composition of matter consisting of a compound of sodium phosphate, sodium nitrate and sodium hydroxide.

8. The herein described composition of matter consisting of a compound of sodium phosphate, sodium chloride and sodium nitrate, free sodium hydroxide of the sodium phosphate. 76
9. The herein described alkaline composition of matter which consists of sodium phosphate-sodium nitrate. 76
10. The herein described composition of matter of crystalline form consisting of 41% to 43.6% trisodium phosphate, 5.55% to .08% sodium nitrate, and 0.22% to 2.10% sodium hydroxide and water of crystallization. 76
11. The herein described composition of matter of crystalline form consisting of sodium phosphate, a plurality of salts of monobasic acids, sodium hydroxide and water of crystallization. 80
12. The herein described process of manufacture of a sodium phosphate-sodium nitrate compound which includes the steps of dissolving sodium phosphate and sodium nitrate in water at an elevated temperature to produce a mother liquor having an alkaline ratio of approximately 1 and crystallizing sodium phosphate-sodium nitrate crystals from the mother liquor. 85
13. The herein described method of manufacturing sodium phosphate-sodium nitrate compound, which includes the steps of dissolving sodium phosphate and a large excess of sodium nitrate in water at an elevated temperature to produce a mother liquor having an alkaline ratio of approximately 1, and crystallizing sodium phosphate-sodium nitrate crystals from the mother liquor. 90
14. The herein described process of manufacturing trisodium phosphate-sodium nitrate compound, which includes the steps of dissolving trisodium phosphate, disodium phosphate and an excess of sodium nitrate in water at an elevated temperature, and crystallizing sodium phosphate-sodium nitrate crystals from the mother liquor. 95
15. The herein described process of manufacture of a sodium phosphate-sodium nitrate compound, which includes the steps of dissolving a sodium phosphate and a plurality of salts of monobasic acids in water, one of which salts of monobasic acids is a sodium nitrate salt, at an elevated temperature to produce a mother liquor having an alkaline ratio of approximately 1, and crystallizing from the mother liquor crystals of salts containing sodium phosphate and the salts of the monobasic acids. 100
16. The herein described process of manufacture of a sodium phosphate-sodium nitrate compound, which includes the steps of dissolving a sodium phosphate including free sodium hydroxide and sodium nitrate in water at an elevated temperature, and crystallizing from the solution sodium phosphate-sodium nitrate crystals wherein the sodium nitrate has replaced a portion of the 105
- 110
- 115
- 120
- 125
- 130